

## UNITED STATES PATENT OFFICE

GEORGES DE NIEDERHÄUSERN, OF BASEL, SWITZERLAND, ASSIGNOR TO THE FIRM OF  
DURAND & HUGUENIN S. A., OF BASEL, SWITZERLAND

## PRODUCTION OF FAST DYEINGS WITH ESTER-SALTS OF LEUCO VAT-DYEESTUFFS

No Drawing. Application filed April 19, 1929, Serial No. 356,621, and in Germany April 26, 1928.

From the ester-salts of the leuco vat-dye-stuffs (indigosols, see U. S. patent specification No. 1,448,251) the original vat-dyestuffs can be re-formed through acid oxidation.

- 5 On this fact is based a dyeing process which has various forms of application and consists in principle in bringing such an ester-salt (indigosol) on to the fibre and then developing the dyeing on the latter by acid oxidation  
10 10 (re-formation of the dyestuff, see U. S. patent specification No. 1,575,958).

It has now been found that the development of ester-salts of leuco-vat-dyestuffs compared with the hitherto known processes can be simplified and improved, since the surprising observation has been made, that the said ester-salts (Indigosols) can be developed on the fibre under the action of water soluble cupric salts in the presence of an organic acid, being  
20 not injurious to the fibre, and other suitable ingredients, by means of a simple drying operation. The drying process may be conducted at ordinary temperature or at a raised temperature; in the former case, the development of the dyeing proceeds more slowly than in the latter case.

It is not excluded that in the case of this oxidation with copper salts the oxygen of the air takes a part, the copper salts having probably also the function of a catalyst.

The indigosols may be brought on to the fibre by a printing or padding operation together with a cupric salt and also with an agent acting as an acid. Another method is to first impregnate the fibre with a cupric salt and subsequently to print the indigosol together with an acid. Through drying, advantageously at a temperature of 50-70° C.,  
35 35 the dyeing is quickly and smoothly developed. The proportion of cupric salt to be used depends on the proportion of indigosol employed.

Certain auxiliary ingredients, such as for  
45 instance ethylenethioglycol, diethyleneglycolmonoethyl ether etc. promote or favor the operation of development.

The new process may be illustrated by the following examples, the parts being by  
50 weight:—

## Example I

A cotton piece is padded in a solution of:

|                          | Parts  |
|--------------------------|--------|
| Copper sulphate crystals | 5 55   |
| Tragacanth thickening    | 15     |
| Formic acid              | 5      |
| Water                    | 225    |
|                          | 250 60 |

then wrung out and dried. The material thus prepared is then printed with a printing colour consisting of:

|                                                      | Parts   |
|------------------------------------------------------|---------|
| Ester-salt of 4:4'-dimethyl-6:6'-di-chlorothioindigo | 65 3.6  |
| Ethylenethioglycol                                   | 5       |
| Diethyleneglycolmonoethyl ether                      | 5       |
| Tragacanth thickening                                | 60      |
| Water                                                | 26.4 70 |
|                                                      | 100     |

It is then dried, washed and soaped at the boil, whereby the dyeing is completely developed; in this way, bright, fast prints are obtained.

## Example II

A cotton piece is padded in the following solution:

|                          | Parts |
|--------------------------|-------|
| Copper sulphate crystals | 10    |
| Water                    | 176   |
| Tragacanth thickening    | 10    |
| Formic acid              | 4 85  |
|                          | 200   |

The material is then dried and printed with a printing colour consisting of:

|                               | Parts |
|-------------------------------|-------|
| Ester-salt of tetrabromindigo | 5     |
| Ethylenethioglycol            | 10    |
| Tragacanth thickening         | 55    |
| Lactic acid                   | 2     |
| Water                         | 28 95 |
|                               | 100   |

and thereupon dried at a temperature of about 70° C. Through this drying, the dyeing is smoothly and completely developed.

The material is finally washed and soaped at the boil.

*Example III*

5 The fibre is padded in a solution containing:

|                                                       | Parts |
|-------------------------------------------------------|-------|
| Ester-salt of 6:6'-diethoxythioindigo                 | 3     |
| Diethyleneglycolmonoethyl ether                       | 5     |
| Tragacanth thickening                                 | 5     |
| 10 Copper sulphate, solution of 10 per cent strength  | 10    |
| Ethylene thioglycol, solution of 10 per cent strength | 1     |
| Formic acid                                           | 2     |
| 15 Water                                              | 74    |
|                                                       | 100   |

then wrung out and dried at about 70° C.

20 The completely developed dyeing is then washed and soaped at the boil.

*Example IV*

Cotton is printed with the following printing colour:

|                                                                     | Parts |
|---------------------------------------------------------------------|-------|
| Ester-salt of 6:6'-dichlor-7:7'-dimethylthioindigo                  | 6.6   |
| Ethylene thioglycol                                                 | 4     |
| Water                                                               | 15.4  |
| 30 Starch and tragacanth thickening                                 | 50    |
| Then the whole is cooled down and when cold there is added thereto: |       |
| Lactic acid                                                         | 4     |
| 35 Copper sulphate, solution of 10 per cent strength                | 20    |
|                                                                     | 100   |

40 The material is thoroughly dried, preferably on drying cylinders. The completely developed prints are then washed and soaped at the boil.

In place of copper sulphate used in these examples, another cupric salt, such as for instance copper chloride, may be used to give the same results.

In this process ester-salts of all classes of vat-dyestuffs, such as those of the indigo, thioindigo, anthraquinone, quinone anilid series and so on can be employed.

What I claim is:—

1. A process for producing fast dyeings 75 with ester salts of leuco-vat-dyestuffs, which consists in applying on the fibre an ester salt of a leuco-vat-dyestuff together with a cupric salt and an organic acid not injurious to the fibre, and performing the development by a 80 simple drying operation.

2. A process for producing fast dyeings 85 with ester salts of leuco-vat-dyestuffs, which consists in applying on the fibre an ester salt of a leuco-vat-dyestuff together with a cupric salt and an organic acid not injurious to the fibre, and performing the development by a simple drying operation at temperatures of 50-70° C.

3. A process for producing fast dyeings 90 with ester salts of leuco-vat-dyestuffs, which consists in applying on the fibre the ester salt of a leuco-vat-dyestuff together with cupric sulphate and an organic acid not injurious to the fiber, and performing the development by a 95 simple drying operation.

4. A process for producing fast dyeings 100 with ester salts of leuco-vat-dyestuffs, which consists in applying on the fibre the ester salt of leuco-6:6'-diethoxythioindigo together with a cupric salt and an organic acid not injurious to the fibre, and performing the development by a simple drying operation.

In witness whereof I have hereunto signed my name this 6th day of April 1929.

GEORGES DE NIEDERHÄUSERN.

110

115

120

130